

## UNITED STATES PATENT OFFICE

ERNEST H. HUNTRESS, OF MELROSE, MASSACHUSETTS, ASSIGNOR TO PLYMOUTH CORDAGE COMPANY, OF PLYMOUTH, MASSACHUSETTS, A CORPORATION OF MASSACHUSETTS

## INCHOATELY MARKED ARTICLES OF MANUFACTURE

No Drawing.

Application filed February 29, 1928. Serial No. 258,134.

This invention relates to improvements in inchoately marked articles of manufacture. More particularly it relates to the provision of a distinguishing device for a manufactured product of any sort that is not readily capable of being durably and distinctively marked by ordinary methods. The purpose is to provide so that the authenticity or identity of a particular specimen of the product

10 may be determined, to authenticate or identify it as being of a certain origin, or as being made by a particular formula, or as having any other specific attribute which the device, if present, is known to signify, notwithstanding 15 that the specimen under examination has passed out of the hands of its maker into commerce, and even may have passed through its industrial life to the verge of destruction.

The invention will be herein described as it 20 may be applied in connection with rope, this being a particular article of manufacture in which the utility of such a device is especially prominent, and for which the invention has been experimentally tested and found successful. The customary marking device for 25 identifying a rope, viz., the introduction of a distinctively colored yarn, has become so common, so readily counterfeited and so open to challenge as to its authenticity, that such 30 yarns have ceased to be a satisfactory marking means.

For the needed invention to be of the desired practical value, the technique of practicing it must be simple, reliable and economical. That is, it should be capable of being performed quickly and by unskilled workmen; without complication of apparatus or of chemical manipulation; and without serious interruption of or addition to the existing 35 manufacturing processes for the article to which it is to be applied. It must be reliable both in the sense of giving results which are constantly reproducible, under ordinary industrial conditions, and also in the sense that 40 the production of the ultimate results must not be impaired either by the deterioration which is incidental to age of the rope, nor by exposure of the rope to the usual incidents such as repeated flexure, abrasion, and gathering of dirt or absorption and evaporation

of water, oil or gasoline; and it must on the other hand be of such a nature that the characteristic results cannot be produced by other materials which may naturally be introduced into rope for special purposes, such as for lubrication, for water-proofing or for mildew-proofing. Obviously it is requisite that the treatment should not harm the strength or other qualities of the fibres or other material treated.

The invention, by the preliminary impregnating of a yarn, provides in the completed rope a permanent inchoate mark which remains for any desired period during the marketing, industrial use and other life of the rope, until by the application of a suitable chemical reagent the inchoate mark becomes a finished mark of distinctive color aspect and of permanent character. In the form of the invention herein described, which is particularly useful where the attribute of secrecy is desired, the inchoate form of the mark does not noticeably affect the appearance, the feeling or other characteristics of the yarn to which it is applied; and the inchoate mark is indistinguishable by ordinary inspection of the rope.

In the particular method and materials here described for illustrating the invention the fundamental principle is that the color is produced in the fibre of the yarn by chemical reaction between two separate substances, one of which is already fast in the fibre. The rope is completed and becomes an article of commerce and of industrial use with the application of only the first component. This rope is a completely identifiable product. The particular system to which resort is had for producing color by reaction, in the illustration here given, is the use of a developed azo dye or "ice color." In the general practice of this system of dyeing, i. e., in the dyeing of fabrics, the color is produced by the interaction in alkaline solution of an alkali salt of a phenolic body with an aromatic amine in solution, which has been diazotized. The chemical reaction is complicated and difficult to carry out; the phenol has to be preliminarily applied to the fibre and dried thereon and then the developer or second

component applied practically immediately or else the coloring of the fibre will be feeble, or fail altogether. The present invention proposes to use, for the first component of the 5 dye, a substance which has such an affinity for the fibre that by adsorption, penetration of the fibre cells, or otherwise, it adheres permanently. For this the arylamides of 2, 3 hydroxynaphthoic acid are available. And 10 instead of the difficult development above mentioned, involving the diazotizing of the second component, the invention is practical for use in the field, without laboratory or dye-room equipment, and without the skill of a 15 chemist or the technique of a dyer, so that an unskilled person can detect the presence of the inchoate mark, because it employs as developer a salt which is especially prepared in permanently diazotized form. This may be 20 one of the alkali salts of the nitrosamines of primary aromatic amines. In the present invention it is a unique feature that the combination of the first and second components of the dye does not occur during the preparation 25 of the marker yarn, but is caused to take place only after the rope is complete and on an occasion in which all of the other yarns as well as that which is inchoately marked are together immersed in a solution, 30 the second component, to which the inchoately marked yarn immediately responds by acquiring a color strikingly distinctive from that of the solution and from that which itself and the other yarns previously had and 35 from that which the other yarns acquire by being immersed in the solution. The first component is here used therefore only to impregnate permanently the marker yarn, and preferably not to impart color or to produce 40 any other visible change therein, and the second component is used months or years later to detect the presence of the first. The arylamides of 2, 3 hydroxynaphthoic acid, suggested as the first component, are available 45 commercially as "AS Naphthols." Their importance for the present invention over all other types of phenols or naphtholic substances is due to their unique property of possessing great affinity for the fibres, such as 50 manila, sisal, etc., used in rope, before the formation of any azo dye stuff by reaction with the second component has taken place. The alkali salts of the nitrosamines of primary aromatic amines, suggested as the second component, are available commercially 55 as "Fast Salts", the term "fast" signifying the rapidity with which they work. The other yarns of the rope, not having been treated with the phenol, do not respond to 60 the application of the Fast Salt, and remain unchanged in aspect, except for a slight color which they may acquire from the initial color of the solution of Fast Salt in water. This last is not the finished color produced by 65 the reaction of the Fast Salt with the phenol.

It will thus be perceived that the invention by which the foregoing results are attained is a species of the generic improvement which consists, in the case of rope, in providing a 70 yarn which reacts differently from the way in which the other yarns react, when all together are subjected to a test treatment.

A description in detail of an illustrative instance of the practice of the invention follows:

The inchoate mark is prepared by brief immersion of an ordinary rope yarn, consisting of manila fibre and containing the usual oil, in a hot water solution, containing, in addition to sulfonated castor oil ("soluble oil") 80 and an excess of free alkali, a small concentration (0.10-0.25%) of an arylamide of 2, 3 hydroxynaphthoic acid. A suitable formula for this solution is indicated by the following:

1.0 g 2-hydroxy 3-naphthoic anilide (Naphthol AS)  
2.0 g soluble oil  
2.0 g 23.5% sodium hydroxide solution  
diluted to 1000 c. c.

This gives a naphthol concentration of 0.109% and a free alkali concentration of 0.03%. Variations may be made. A considerable number of naphthols of the AS series are available and all of the series appear to possess marked affinity for the fibre, this not being limited to manila hemp, but being true of cotton and other; but there is a difference in the deepness of the color ultimately obtained by development, this being greatest with naphthol AS/BO, 2-hydroxy 3-naphthoic alphanaphthalide which has greatest affinity for the fibre, but being satisfactory with naphthol AS which has much less affinity but is less expensive. The concentration may vary. Even at a naphthol concentration of 0.05% and an immersion of ten seconds the color ultimately developed is sufficiently deep to serve as a distinguishing marker. In fact, however, the duration of immersion does not make such difference, the diminution of depth of shade obtained with decreasing time of immersion being not considerable, in the solution of lower concentration, whether the immersion were sixty seconds or two seconds. The rate of penetration of the naphthol into the fibre increases with temperature. The use of soluble oil maintains a satisfactory homogeneity of solution and during the preparation of the naphthol solution its presence markedly facilitates the mixing of the dry powder with the alkali. Its presence however does not affect the ultimate color produced nor perceptibly increase the natural penetrating power of the alkaline solution. The presence of excess alkali prevents hydrolysis of the naphthol salt and resultant precipitation of the free naphthol itself; but if the alkali be present in excess of a certain minimum representing alkali equivalent to 120

the naphthol used, the degree of its excess does not appear to affect the shade of color developed. The deleterious effect of the free alkali on the fibre has been found to be entirely negligible as shown by tensile strength tests. When thus impregnated some of the AS naphthols possess so great an affinity for the rope fibre that even after short pieces of made up rope containing the impregnated 5 yarn had been shaken for one hundred hours with sea water or ordinary water the inchoate marked yarn still responded satisfactorily to the developing treatment. The inchoate mark is made by the simple process 10 for running a regular yarn which is later to be incorporated in the rope, or other article, that is to be marked, through a bath of the above solution or such variation of it as may be desired, with such brief period of 15 immersion as may be found convenient. Preferably this yarn will be allowed to dry before it is incorporated in the rope, in order to prevent the solution which is wet upon it from being to some extent transferred to a 20 neighboring yarn as would happen if it were incorporated in the rope while wet, but the drying is not a necessary part of the process of rendering the yarn sensitive to development into a permanent color. A rope having 25 been made according to ordinary or any suitable method, or the other article, whatever it may be, having been made, incorporating one or more of the treated yarns or other elements, the article is complete and goes into 30 commerce and industry. In the greater number of instances in practical life this is as far as the article will ever go toward having a mark of the nature under discussion. The complete article is characterized by having 35 the mark in inchoate condition.

In any instance in which it is desired, and at any period of time afterward, even years, and in any place however remote from factory or laboratory, the inchoate mark may 40 be developed into a finished mark. Under laboratory conditions it is possible to carry out the development by the use of diazotized solution of m-nitro p-toluidine base as developer, the diazonium salts being obtained 45 by the carefully regulated action of nitrous and hydrochloric acids upon the various color bases. But for practical commercial and industrial life wherein convincing and certain and quick test is requisite, which can be applied 50 by a person unskilled in chemistry or in the technique of dyeing, it is preferable to use for the developer a stabilized form of these diazonium salts, such being obtainable commercially, among materials used for 55 manufacturing azo dyes, as colored powders which are easily soluble and in addition to the actual diazonium salts contain a large quantity of some inorganic material such as zinc chloride which effects the stabilization 60 of the materials. One commercial variety

is known under the commercial name of "Fast Salts", further designated usually by some color as red, orange, scarlet, blue, black. The development of the inchoate marker to the color produced by the particular dye stuff 70 can then be effected by dissolving a little of the developer in a tumbler of water, and immersing an end of the rope in the solution. The color appears in a few seconds, in the 75 yarn which is the inchoate mark, the other yarns remaining unaffected by the characteristic reaction, although there may be a slight change of color in another direction. For example, upon using an inchoate marker prepared by impregnation resulting from ten 80 seconds immersion in a 0.10% naphthol AS solution containing 0.18% sodium hydroxide and 1% soluble oil, and using Fast Blue Salt B (a chemical name for which is stabilized tetrazotized dianisidine) for development, 85 satisfactory results are obtained, whether the strength of developing solution was 1% or even 0.01%, the rapidity of development being greater with the more concentrated solution. Using a marker impregnated with 90 1.4% AS/BO solution, and developing with 1% Fast Salt Blue B solution the marking yarn acquires a deep reddish blue, while the other yarns in the rope at the same time change from their characteristic hemp color 95 to a pale pink, giving excellent contrast.

If it were desired that instead of this element of secrecy there should be an indication as to which is the treated yarn the invention can equally be applied. For example, the marker yarn might be preliminarily dyed some distinctive color or might be distinguished by difference of material; or might be simultaneously dyed distinctively by a dye suitable for that purpose and impregnated by 100 the naphthol AS solution, but in this case it would be desirable to choose a dye having an affinity for the fibre approximating that of naphthol AS so as to get a smooth color.

Rope thus made, by any of the formulae 105 first above given, is found to contain an inchoate marker which is highly resistant to water, sea water, boiling gasoline, hot mineral oil and other deleterious influences which a rope may encounter during its industrial life.

A combined or double and confirmatory marking is possible to be obtained in a single 110 yarn by the use of the present invention by the selection of a naphthol, for example naphthol AS/BR (a chemical name for which is Beta-hydroxy-naphthoic acid dianisidine) which particular naphthol possesses a very brilliant yellow fluorescence in ultra violet light, although another naphthol, as for example, naphthol AS/BS shows no fluorescence while others show a pale yellow fluorescence of no particular importance.

In the rope or other article which is marked 115 the developed marker herein described may

be associated with ordinary or other markers, embodied in other yarns, the use of which is not precluded, and the aspect of which does not undergo the characteristic change when 5 immersed in the developing solution.

While the disclosed herein as it may be applied to a yarn of rope, by impregnation of the yarn through an immersing of it in solution, the invention is not limited to that material nor to that method of application of the 10 solution or the developer.

It is intended that the patent shall cover by suitable expression in the appended claims, whatever features of patentable novelty exist 15 in the invention herein disclosed in relation to the provision of an inchoate mark and its development into a finished mark.

The invention claimed is:

1. A new article of manufacture consisting 20 of an industrial product having incorporated therein, in undeveloped form, a developable naphthoic substance the characteristics of which constitute potential identifying means and include a strong affinity for the 25 material of the product in which it is incorporated, said undeveloped naphthoic substance being capable, despite the lapse of a long period of time, of manifesting its presence by reacting chemically into developed 30 form.

2. A new article of manufacture consisting 35 of an industrial product having incorporated therein, in undeveloped form, a developable naphthoic substance the characteristics of which constitute potential identifying means and include a strong affinity for the material of the product in which it is incorporated, said undeveloped naphthoic substance being capable, despite the lapse of 40 a long period of time, of manifesting its presence by reacting chemically into developed form when brought into contact with a diazotized reactant.

3. A new article of manufacture comprising 45 an industrial product having incorporated therein, in undeveloped form, one of the aryl amides of 2, 3 hydroxynaphthoic acid, the characteristics of which amide constitute potential identifying means and include a 50 strong affinity for the material of the product in which it is incorporated; said undeveloped amide being capable, despite the lapse of along period of time after its being so incorporated, of manifesting its presence in 55 said product by reacting chemically into developed form when brought into contact with a diazotized reactant.

Signed at Boston, Massachusetts, this thirtieth day of January 1928.

60 ERNEST H. HUNTRESS.